

## UNITED STATES PATENT OFFICE.

OSCAR LÖW-BEER, OF FRANKFORT-ON-THE-MAIN, GERMANY, ASSIGNOR TO CHEMISCHE FABRIKEN WORMS A. G., OF FRANKFORT-ON-THE-MAIN, GERMANY, A CORPORATION OF GERMANY.

TANNING MATERIAL CONTAINING ALKALI-EARTH METALS AND HEAVY METALS AND PROCESS OF MAKING SAME.

No Drawing.

Application filed March 30, 1921. Serial No. 457,139.

To all whom it may concern:

Be it known that I, OSCAR LÖW-BEER, a citizen of the Czechoslovakian Republic, residing at Frankfort-on-the-Main, Germany, <sup>5</sup> have invented certain new and useful Improvement in Tanning Materials containing Alkali-Earth Metals and Heavy Metals and Processes of Making Same, of which the following is a specification.

10 My present invention relates to a process of preparing tanning substances and of tanning animal hides.

Hitherto artificial tanning substances obtained by coupling organic compounds <sup>15</sup> either directly with each other or by atoms or by atomic groups (see German Patents Nos. 265,855, 266,139, and 280,233) have been used for tanning animal hides. According to the specifications of these patents <sup>20</sup> such tanning substances or mixtures thereof with other tanning—or non-tanning materials,—which however merely constitute mechanical mixtures,—can only be used in acid solution. The said specifications do <sup>25</sup> not contain any statements as to employing the respective substances in neutral solution, from which it must be concluded that they are intended to be used only in the usual acid solution. Moreover, neither the artificial tanning substances above referred to <sup>30</sup> nor the alkali metal salts derived therefrom possess in neutral solution (tested on Congo paper) the character of a tanning agent and do not precipitate animal glue.

35 Now I have made the surprising observation that salts can be formed from tanning substances produced by the chemical reaction of artificial tanning materials consisting of organic components coupled with <sup>40</sup> aluminium or chromium compounds and having the general formula



45 whereon X stands for an aliphatic radical or an aromatic radical, Y for another radical as for instance another aliphatic radical or another aromatic radical, Z for a connecting link, such as an atom or atomic group and Me for an alkaline earth metal or a heavy metal, which precipitate glue copiously in a <sup>50</sup> solution neutral to Congo paper suitable for

tanning animal hides. The use of such <sup>55</sup> solutions for tanning hides has the great advantage that the injurious action of the acids which, if not washed out of the finished leather, gives a leather which becomes cracked is avoided and that the onerous washing out of the finished leather which <sup>60</sup> impairs the yield of the leather can be dispensed with.

The tanning action of the above mentioned salts of tanning substances which yield solutions neutral to Congo paper has <sup>65</sup> hitherto been unknown and in view of the behaviour of the corresponding alkali metal salts this action could not be foreseen, otherwise the above-mentioned German specifications would certainly have particularly <sup>70</sup> pointed out their formation and application in view of the great advantages to be derived therefrom.

The process for preparing said tanning salts which yield solutions neutral to <sup>75</sup> Congo paper may be advantageously carried out as set forth in the following examples:

Example 1.—150 kilos of coal tar oil are sulfonated with 150 kilos of sulfuric acid <sup>80</sup> of 98 per cent strength and the product is carefully condensed with 45 kilos of a formaldehyde solution of 40 per cent strength first at a temperature of 40–60° C. and finally at 75° C. After the mass has <sup>85</sup> become stiff it is dissolved by introducing steam. The excess of sulfuric acid is then neutralized by means of potash solution until the liquid is only faintly acid whereupon aluminium hydroxid is added until a test <sup>90</sup> does not change the color of Congo paper. The solution thus obtained may be used directly for tanning, it shows on litmus paper an acid reaction, on Congo paper a neutral reaction and precipitates glue freely with a <sup>95</sup> grey color. The dry substance obtained by evaporation chars when heated, without previously melting and is insoluble in ether and benzene.

Example 2.—100 kilos of coal tar phenols <sup>100</sup> of melting point 185–200° C. are mixed with 275 kilos of crystallized sodium sulfite, 275 litres of water and 150 lbs. of a formaldehyde solution of 30 per cent strength and this mixture is heated in an <sup>105</sup> autoclave for about 8 hours at 140–150° C.

The condensation mass is acidified by means of sulfuric acid and the sulfurous acid is boiled out. The product is then neutralized with chromium oxide hydrate until it does no longer change the color of Congo paper. The solution shows on litmus paper an acid reaction, but on Congo paper a neutral reaction; it precipitates glue with a brownish color. The dry substance chars when heated, without first melting; it is soluble in water but insoluble in ether and benzene.

*Example 3.*—75 kilos of naphthalene and 75 kilos of phenol are sulfonated for 8 hours at 120° C. with 150 kilos of sulfuric acid of 98 per cent strength and the product is condensed at 60–80° C. with 75 kilos of a formaldehyde solution of 30 per cent strength until a test with a glue solution shows no further increase of the precipitate. The mass thus obtained before getting stiff is diluted with 100 litres of water, neutralized with calcium hydroxide until it shows only a slightly acid reaction and is then filtered. Into the solution basic chromium sulfate is introduced until it does not change the color of Congo paper; it shows on litmus paper an acid reaction, on Congo paper a neutral reaction and precipitates glue with a brown color. The dry substance chars when heated, without melting; it is soluble in water, insoluble in ether and benzene.

*Example 4.*—100 kilos of creosote oil are sulfonated with 150 kilos of sulfuric acid of 98 per cent strength and the product is condensed as indicated in example 3 with 45 kilos of a formaldehyde solution of 30 per cent strength. The reaction mass is diluted with water and mixed with a solution of 150 kilos of chromium sulfate and 200 kilos of caustic soda solution of 40° Bé. The tanning liquor thus obtained gives an acid reaction on litmus paper, but a neutral reaction on Congo paper and it precipitates glue with a greyish-green color. The dry substance chars when heated, without previously melting and is insoluble in ether and benzene.

*Example 5.*—75 kilos of naphthalene and 75 kilos of phenol are sulfonated as indicated in example 3 with 150 kilos of sulfuric acid of 98 per cent strength and then condensed with 75 kilos of a formaldehyde solution of 30 per cent strength. The reaction mixture obtained before getting stiff is diluted with 100 litres of water and after adding thereto 50 kilos of tanning it is coupled at 70–80° C. with 50 kilos of a formaldehyde solution of 30 per cent strength. There are then introduced 85 lbs. of potash solution of 36° Bé. and the whole is neutralized with aluminium hydroxide until a test on Congo paper does not change its color. The solution shows a neutral reaction and precipitates glue with a grey color; the dry

substance has the same properties as that obtainable according to example 4.

*Example 6.*—23 kilos of 2,6 naphtholsulfonic acid are mixed with a solution of 18 kilos of glucose in 10 litres of water and this mixture is subjected to reaction at water-bath temperature with 10 kilos of a formaldehyde solution of 30 per cent strength. The product is dissolved in hot water, filtered and chromium hydroxide is added thereto until a test on Congo paper does not change the color of the latter. The solution shows on litmus paper an acid reaction, on Congo paper a neutral reaction, and precipitates glue with a greyish green color. The dry substance does not show any melting point, but gets charred when heated and is soluble in the aforementioned organic solvents.

The hereinbefore described neutral tanning substances are soluble in water and possess the properties of the usual tanning agents; they can be employed alone or mixed with other tanning agents or other ingredients and they are alone suitable for the combined tannings process. If the aqueous solutions of the hereinbefore or hereinafter described tanning substances are strongly diluted there is a separation of flakes which can however be prevented by adding suitable bodies such as for instance, waste liquor from sulfite cellulose or its metallic compounds.

The process for tanning leather by means of the before-mentioned salts of tanning substances which give on Congo paper a neutral reaction, can be carried out in the following manner:

The prepared unhaired skin is treated with a tanning liquor of 2–3% strength of the tanning substances composed as indicated in examples 1–6. The tanning is effected according to the kind of skin, in tan pits, in the reel or in the fulling trough, the strength of the liquor being adjusted and the duration of tanning modified accordingly.

It has been proved that when employing the above described process the unhaired skins can without being previously heated be tanned directly in the vat in a short time without fear of producing a leather having a rough grain.

In the place of the above-described artificial tanning agents produced from coupled organic compounds and aluminium or chromium compounds, there may be obtained other new tanning substances by treating the same with compounds of other heavy metals, which new tanning substances have also the advantage of strongly precipitating glue in a solution neutral to Congo paper, of tanning animal hides and of being soluble in water.

Such heavy metal compounds are for in-

stance cerium hydroxide, stannous chloride, cerium sulfate and the like.

Further experiments made along the lines of my above mentioned observations have proved that such artificial tanning substances may also be coupled with compounds of heavy metals with the formation of basic metal salts which possess the advantage that during the tanning process 10 relatively larger quantities of heavy metals are deposited in the animal hides. The new products consequently constitute complex compounds of basic metal salts possessing the further advantageous property of tanning animal hides in a solution neutral to Congo paper.

The tanning with these new tanning substances is also carried out, according to the kind of unhaired skin, in tan pits, in the reel 20 or the fulling trough, the strength of the liquor being adjusted and the duration of tanning modified accordingly. These compounds of tanning substances possess the properties of the ordinary tanning agents 25 and can be employed alone or mixed with other suitable ingredients and they are also adapted for the combined tanning process.

*Example 7.*—100 kilos of coal tar phenols of melting point 185-200° C. are mixed 30 with 275 kilos of crystallized sodium sulfite, 275 kilos of water and 150 kilos of a formaldehyde solution of 30 per cent strength and this mixture is heated in an autoclave for 8 hours at 140-150° C. The condensation mass is acidified by means of sulfuric acid and the sulfurous acid is boiled out. The product is then neutralized by means 35 of cerium hydroxide until a test on Congo paper does not show any change of color. 40 Its solution gives on litmus paper an acid reaction, on Congo paper a neutral reaction and precipitates glue with a brown color. The dry substance chars when heated while 45 strongly puffing up without previously melting; it is readily soluble in water but insoluble in ether and benzene.

*Example 8.*—75 kilos of naphthalene and 50 kilos of phenol are sulfonated with 150 kilos of sulfuric acid of 98 per cent strength and the product is condensed with 75 kilos of a formaldehyde solution of 30 per cent strength. The reaction mixture thus obtained before getting stiff is diluted by adding 100 litres of water and after addition 55 thereto of 50 kilos of tannin it is coupled at 70-80° C. with 50 kilos of a formaldehyde solution of 30 per cent strength. There are then introduced 85 kilos of potash solution of 36° Bé. and cerium hydroxide added to the whole until a test does not 60 change the color of Congo paper. The solution shows on litmus paper an acid reaction, on Congo paper a neutral reaction and it precipitates glue with a brownish coloration. The dry substance when heated on

a spatula chars without previously melting; it is readily soluble in water, insoluble in ether and benzene.

*Example 9.*—75 kilos of naphthalene and 75 kilos of phenol are sulfonated at 120° 70 C. for 8 hours with 150 kilos of sulfuric acid of 98 per cent strength and the product is condensed with 75 kilos of a formaldehyde solution of 30 per cent strength until a test with a glue solution does not show 75 any further increase of the precipitation. The mass thus obtained before getting stiff is diluted with 100 litres of water, neutralized with calcium hydroxide and filtered while hot. The resulting product is treated 80 with sodium carbonate and the calcium carbonate is filtered off. The solution of the metal salt of the tanning substance is then run while stirring into a solution of chromium chloride containing about 2 molecular 85 proportions of chromium chloride calculated upon one molecule of the tanning substance, whereupon sodium carbonate is added for forming the basic salt until all of the hydrochloric acid is linked to sodium. 90 The solution shows on Congo paper a neutral reaction and when mixed with animal glue it gives a copious precipitate. The dry substance when heated chars without previously melting; it is soluble in water, but insoluble 95 in ether and benzene.

Instead of chromium chloride, other heavy metal compounds can be combined with artificial tanning substances so as to obtain the corresponding salts, and the reaction may of course also be effected by any other known process for the formation of basic salts.

Finally there may also be used for tanning animal hides alkaline earth metal salts 100 of the above described tanning substances consisting of coupled organic components. Such salts possess likewise the property of tanning animal hides in solutions neutral to Congo paper, a fact hitherto unknown 105 and upon which the forementioned advantages depend.

As is known, calcium compounds and the like are used with reluctance in tanneries because in most cases they cause the leather 110 to become brittle, hard and cracky, however, the calcium coupled with the aforescribed artificial tanning substances does not exercise such detrimental action.

In German Patents Nos. 265,855, 266,139, 120 280,233 and 281,484 and in Austrian Patent No. 69,194 are described artificial tanning substances consisting of coupled components to be used alone or mixed with other tanning or non-tanning materials but in these 125 patents no reference whatever is made to a chemical conversion of the respective compounds into alkaline earth metal salts capable of tanning in solutions neutral to Congo paper, but they only deal with mere 130

mechanical mixtures of different bodies. The new products precipitate animal glue, are soluble in water and possess the properties of the ordinary tanning substances; they 5 can be employed alone, or mixed with other tanning agents or other ingredients and they are also adapted for the combined tanning processes.

*Example 10.*—The prepared unhaired skin 10 is treated with a tanning liquor of about 2-3 per cent strength, the tanning substance of which has been prepared as follows: 75 kilos of naphthalene and 75 kilos of phenol are sulfonated at 120° C. for 8 15 hours with 150 kilos of sulfuric acid of 98 per cent strength and the product is condensed at 60-80° C. with a formaldehyde solution of 30 per cent strength until a test with a glue solution does not show any 20 further increase of the precipitate. The mass thus obtained before getting stiff is diluted with 100 litres of water, neutralized with calcium hydroxide and filtered while hot. The solution thus obtained can be 25 used for tanning or it may be evaporated to dryness. The tanning operation is carried out, according to the kind of skin, in the tan pit, in the reel or in the fulling trough, the strength of the liquor and the duration 30 of the tanning being adjusted accordingly.

*Example 11.*—The tanning is effected as indicated in example 1, with a tanning substance prepared as hereafter described:— 35 100 kilos of coal tar phenols of melting point 185-200° C. are mixed with 275 kilos of crystallized sodium sulfite, 275 litres of water and 150 kilos of a formaldehyde solution of 30 per cent strength and the whole is heated in an autoclave for about 8 hours 40 at 140-150° C. The product of the condensation is acidified by adding sulfuric acid and the sulfurous acid is boiled out. The resulting product is neutralized by means of calcium hydroxide until a test on Congo paper shows no change of color, whereupon 45 it is filtered.

*Example 12.*—The tanning is effected by means of a tanning substance prepared as follows:—75 kilos of naphthalene and 75 50 kilos of phenol are sulfonated with 150 kilos of sulfuric acid of 98 per cent strength and the product is condensed with 75 kilos of a formaldehyde solution of 30 per cent strength. The reaction mixture before getting 55 stiff is diluted with 100 litres of water and after adding 50 kilos of tannin coupled at 70-80° C. with 50 kilos of a formaldehyde solution of 30 per cent strength. There is then added calcium hydroxide until there 60 is a neutral reaction and the whole is filtered while hot.

*Example 13.*—The tanning liquor is made up with a tanning substance prepared as follows: 23 kilos of 2-6-naphtholsulfuric acid 65 are mixed with a solution of 18 kilos of

glucose in 10 litres of water and this mixture is caused to react at water bath temperature with 10 kilos of a formaldehyde solution of 30 per cent strength. The product is dissolved in hot water, filtered and then is 70 added calcium hydroxide until a test does not change the color of Congo paper.

The duration of all the above described tanning processes is about 24-60 hours according to the thickness of the leather to 75 be obtained. The finished leather shows a lighter color as compared with that tanned with the natural tanning agents and its cut is of an entirely uniform appearance.

Having now described my invention, what so I claim is:

1. As new products, soluble tanning substances having the general formula:



85

in which X stands for an aromatic or aliphatic radical, Y stands for an aromatic or aliphatic radical, Z stands for an aliphatic atomic group, and Me stands for an alkaline earth metal or a heavy metal.

2. As new products, soluble tanning substances having the general formula:



95

in which X stands for an aromatic radical, Y stands for an aromatic or aliphatic radical, Z stands for an aliphatic atomic group, and Me stands for an alkaline earth metal or a heavy metal.

3. As new products, soluble tanning substances having the general formula:



105

in which X stands for an aromatic radical, Y stands for an aromatic radical, Z stands for an aliphatic atomic group, and Me stands for an alkaline earth metal or a heavy metal.

4. As new products, soluble tanning substances having the general formula:



115

in which X stands for an aliphatic or aromatic radical, Y stands for an aromatic radical, Z stands for an aliphatic atomic group, and Me stands for a heavy metal.

5. As new products, soluble tanning substances having the general formula:



125

in which X stands for an aliphatic or aromatic radical, Y stands for an aliphatic or

130

aromatic radical, Z stands for an aliphatic atomic group, and Me stands for a heavy metal.

6. The process of preparing water soluble tanning substances capable of tanning animal hides in Congo neutral solution and having the general formula:

10



in which X stands for an aromatic or aliphatic radical, Y stands for an aromatic or aliphatic radical, Z stands for an aliphatic atomic group, and Me stands for an alkaline earth metal or a heavy metal which comprises condensing an organic sulfonic

acid compound in the presence of formaldehyde and subjecting the condensation product in solution to the action of a nonacid compound of a metal the salts of which have tanning properties until a Congo neutral solution is formed.

7. The process of preparing new tanning agents which comprises condensing organic compounds containing a salt forming group in the presence of formaldehyde, coupling the condensation product with tannin, and treating the coupled product in solution with a compound of a heavy metal until the solution is neutral to Congo paper.

In testimony whereof I hereunto affix my signature.

OSCAR LOW-BEER.